

April 4, 1939.

H. WEHMEIER ET AL

2,152,717

## METHOD OF CASTING IN A CENTRIFUGAL MOLD.

Filed Dec. 22, 1937

Fig. 1.



Fig. 2.



INVENTORS  
Hermann Wehmeier  
Wolfram Ruff  
BY  
Pennie, Davis, Marion & Edmonds  
ATTORNEYS

## UNITED STATES PATENT OFFICE

2,152,717

## METHOD OF CASTING IN A CENTRIFUGAL MOLD

Hermann Wehmeier and Wolfram Ruff, Wetzlar, Germany, assignors, by mesne assignments, to Centrifugal Pipe Corporation, Jersey City, N. J., a corporation of Delaware

Application December 22, 1937, Serial No. 181,168  
In Germany December 24, 1936

2 Claims. (Cl. 22—201)

This invention relates to apparatus for, and an improved method of, centrifugally casting pipe and particularly to the centrifugal casting of iron pipe. In accordance with the method of the invention a powdered material is sprinkled or otherwise suitably applied in a thin layer on the upper surface of the molten metal as it is being fed into the mold, and the stream of molten metal is so guided as it enters the mold that the upper surface or stratum thereof upon which the powdered material was deposited is brought into contact with the mold. In the casting of iron pipe, for example, the layer or stratum of material in contact with the mold suppresses or prevents the chilling of the iron.

The apparatus of the invention comprises means in combination or cooperation with a centrifugal casting machine of the type in which the pouring trough is relatively displaceable with respect to the mold, for sprinkling powdered material onto the upper surface of the metal as it flows through the trough into the mold. The invention also includes an improved pouring trough having a laterally deflected spout which is so shaped that the uppermost stratum of metal flowing through the trough is brought into contact with the mold, forming the outer portion of the pipe and the remaining portion of the metal forms the inner portion of the pipe.

The method of the invention is particularly adaptable to those centrifugal operations in which the material to be cast is supplied by means of a trough which has relative displacement between the trough and mold. In such operations, the powder is applied as by sprinkling a thin layer on the surface of the molten metal, for example, cast iron, as it flows along the trough and into the mold. The sprinkling may be effected by any suitable mechanical means which is preferably mounted outside of the mold. The apparatus may be mounted on or adjacent the pouring trough or on that part of the machine which carries the mold.

In order that the stream of metal issuing from the trough, or spout of the trough, may contact the wall of the mold with its uppermost, powder-carrying stratum first, it is advantageous to construct the discharge spout of the pouring trough in a particular manner, for example, by means of a prominent rounding-off of the overflow edge of the spout, so as to bring about a deflection of the metal stream sideways and downwardly, in which event the lowermost stratum of the stream can be deflected relatively to the uppermost stratum.

The method of the invention is particularly adapted for the casting of pipe in cooled metallic centrifugal molds. It may, however, be applied to centrifugal casting in other types of centrifugal molds such as sand or refractory lined molds. The method is particularly advantageous in the manufacture of small diameter pipes, although it may be practiced with equal advantage in the centrifugal casting of large-diameter pipes.

In practicing the method of the invention in casting iron pipe, a suitable inert powdered material, such as powdered sand or infusorial earth, or a reactive metallic material such as ferro-silicon, manganese-silicon, ferro-phosphorus, or calcium, magnesium or aluminum alloys may be used. Ferro-silicon is especially efficacious both from a standpoint of technical and economical considerations. In using a metallic or reactive material, for example, ferro-silicon, an especially intense effect on the casting is obtained, presumably due to the preheating of the ferro-silicon powder during its floating on the surface of the molten iron which causes the reaction velocity to be considerably increased. It is possible, when using powdered ferro-silicon, to cast iron pipe in water-cooled centrifugal molds having an inner diameter of 40 mm. and a wall thickness of 4 mm. that are "grey" throughout their entire cross-section.

The powder should be very fine because the finer the powder, the better it floats upon the molten metal in the pouring trough. When an inert material, or a coarse reactive metallic material are used, the powder remains as such on the surface of the metal and is brought into direct contact with the mold, in effect, lining the mold with a coating of the powder. If the powder is a substance which reacts chemically with the iron such as ferro-silicon it may be sufficiently fine that it dissolves in or reacts with the iron before the iron contacts the mold.

In the accompanying drawing,

Figure 1 is a longitudinal section through a centrifugal pipe-casting machine provided with means for practicing the invention;

Figure 2 is a section along line 2—2 of Figure 1.

The mold 1 is rotatably mounted in a longitudinally displaceable carriage 2. The pouring trough 3 extends into the mold, has an inner refractory lining 4, and is mounted on a transversely movable casting carriage 5 which carries a pouring funnel 6 for feeding metal 7 into the pouring trough.

The powder-sprinkling mechanism comprises

a supply receptacle 8, a spreader or sprinkling device 9 and is mounted in such a way that the falling particles of powder are deposited upon the upper surface of the stream of metal 7 flowing along the trough 3 on its way into the mold 1. The sprinkling mechanism may occupy a fixed position relatively to the trough, i. e. it may be rigidly connected with the casting carriage. It may, however, also be attached to carriage 2 so as to participate in its longitudinal displacement, in which case the distance over which the powder is carried becomes progressively smaller. At its discharge end, the trough 3 has a discharge spout 10 bent sideways and downwardly in the direction of rotation of the mold indicated by arrow 11. The overflow edge 12 of the discharge spout is well rounded off.

As will readily be seen in Figure 2, the metal discharged from the spout is so guided or controlled that the uppermost stratum of the stream of metal which carries the powder, or on which the powder was deposited, is brought into contact with the mold wall before the remaining portion of the metal may contact the mold. As a result thereof the action of the powder deposited on the said stratum of metal prevents the pipe being chilled.

We claim:

1. In a method of casting pipe in a centrifugal mold the improvement which comprises sprinkling a metallic powdered material on the upper surface or stratum of the metal as it is being fed into the mold, and guiding the stream of molten metal into the mold in such manner that the said stratum on which the powdered material was deposited is brought into contact with the inner surface of the mold. 10

2. In a method of casting iron pipe in a centrifugal mold in which the metal is poured into the mold by means of a trough which is relatively displaceable with respect to the mold, the improvement which comprises applying powdered material including silicon to the uppermost surface of the metal in the trough, and then guiding the stream of molten metal in such manner that the upper stratum thereof on which the powdered material was deposited is brought into contact with the inner surface of the mold, thereby causing the said stratum to form the outer surface of the pipe. 15 20

HERMANN WEHMEIER. 25  
WOLFRAM RUFF.